# EUROPEAN PATENT SPECIFICATION

(11) **EP 0 430 553 B1**
(45) Date of publication and mention of the grant of the patent: **15.02.1995**
(21) Application number: 90312643.1
(22) Date of filing: 20.11.1990
(51) Int. Cl.: G03G 9/09

(54) **Toner for full colour development**
Toner für totale Farbentwicklung
Toneur pour le développement à pleine couleur

(30) Priority: 20.11.1989 JP 299718/89; 20.11.1989 JP 299719/89; 22.11.1989 JP 301997/89; 22.11.1989 JP 301998/89; 22.11.1989 JP 301999/89; 22.11.1989 JP 302000/89
(43) Date of publication of application: 05.06.1991
(73) Proprietor: MITA INDUSTRIAL CO. LTD., Osaka-shi Osaka-fu 540 (JP)
(72) Inventor: Tsubota, Noriaki, Himeji-shi, Hyogo-ken (JP); Kubo, Masahiko, Yao-shi, Osaka-fu (JP); Fuji, Kazuo, Higashi-osaka-shi, Osaka-fu (JP); Edahiro, Kazuhisa, Hirakata-shi, Osaka-fu (JP)
(74) Representative: Cresswell, Thomas Anthony

(56) References cited:
- EP-A- 0 046 398
- EP-A- 0 275 636
- GB-A- 2 002 913
- GB-A- 2 029 591

## Description

The present invention relates to a toner for full color development where a plurality of toners are overlapped on an image on a copying sheet. More particularly, the present invention relates to a toner for full color development, in which the development characteristics and transfer characteristics are substantially equal in the toners to be overlapped.

Furthermore, the present invention relates to magenta, cyan and yellow toners among toners for full color development. More particularly, the present invention relates to these toners having such an excellent transparency that when these toners are mingled on an image on a transfer sheet, the toners can show the intended colors sharply.

In the fields of the electrophotography and electrostatic printing, toners are used for visualizing electrostatic latent images formed on image carriers. In these toners, a resin having desirable electroscopic and binding properties, for example a styrene resin or a polyester resin, is used as the resin medium, and carbon black or other organic or inorganic coloring pigments are used as the coloring agents.

Full color development in which magenta, cyan, yellow and black color toners are overlapped to form an image has been recently proposed and worked.

In this full color development, a multiple-color original is exposed to light through a color-separating filter. This operation is repeated a number of times using cyan, yellow and magenta color developers and a black toner, and toner images are thus overlapped to obtain a multiple-color image. Organic pigments are used as coloring agents for cyan, yellow and magenta toners used for this full color development, and carbon black is used for a black toner.

Fig. 7 is a diagram illustrating the developing and transfer zones of an image-forming apparatus for obtaining a full color image. In this apparatus, an electrostatic latent image formed on a photosensitive drum 1 by an appropriate means is visualized by a developer in any of the developing devices 3a, 3b, 3c and 3d of a developing unit 2 and is then transferred by a transfer charger 5 onto a transfer material held on a transfer drum 4 by a gripper 6, from which electricity is removed by an electricity-removing charger 7. Furthermore, a toner image developed by a developer in another developing device of the devices 3a, 3b, 3c and 3d is transferred onto the transfer material by the transfer charger, and third and fourth color images are similarly transferred. Thus, a predetermined number of color images are transferred onto the transfer material held on the transfer drum 4, and the transfer material is delivered to a fixing step (not shown) to form a multiple-color image. In general, in the above-mentioned transfer step, an operation of transferring a toner of a different color onto a toner layer transferred on a transfer material is carried out. At this operation, it sometimes happens that the charge of the toner already transferred on the transfer material reduces the working transfer electric field at the transfer of the subsequent toner, and therefore an image having a desired hue cannot be reproduced. For obviating this disadvantage, there is sometimes adopted a method in which the transfer voltage is gradually elevated at the transfer step or the transfer voltage is elevated at the transfer of the third and subsequent toners when the toner layer becomes thick.

However, since the behavior of toners at the practical transfer step is delicate and complicated, even if a predetermined transfer voltage is applied and the value of the transfer voltage is elevated in the later stage, scattering of the toners or insufficient transfer often occurs because the color toners have different characteristics (such as charging characteristics and electric characteristics), and satisfactory results cannot be obtained in the formation of a toner image of a desirable hue.

JP-A-1-32981 proposes a method in which the quantity of the charge of a toner to be developed and transferred is made larger than the absolute value of the already developed and transferred toner to compensate for the reduction of the working transfer electric field and stabilize the transfer operation. According to this method, if it is intended to adopt common development conditions (the charge characteristics of the photosensitive material, the development bias voltage and the sliding contact state between the photosensitive material and the developer carrier), since toners are extremely different in the charge characteristics, development unevenness (insufficient density of the solid portion, thicknening of line and dot images and formation of toner dusts in the peripheral portion of the image area) is caused or scatterring of toners is caused in the machine, and a shear in the hue and fogging are often observed in the formed image.

It is important that color toners should be excellent not only in spectral reflection characteristics but also in spectral transmission characteristics, and if this requirement is not satisfied, an image having a hue similar to the inherent color cannot be obtained. When a full color image is formed by overlapping a plurality of color toners, it is especially important that a transparency should be given to the toners. If color toners having poor transparency are used, the colors of the toners interfere with one another and the formed image becomes dark, and it often happens that an image of a desired color cannot be obtained.

As the means for overcoming the foregoing defects, there have been proposed a method in which a specific fluorine-containing acrylic resin is used as a binder resin medium (JP-A-62-273569) and a method in which an oil-soluble dye such as C.I. Solvent Yellow 60 is incorporated into a yellow toner (JP-A-62-273572).

However, even if these methods are adopted, the original image hue cannot be sharply reproduced by mingling the colors, and it often happens that the formed image becomes obscure and the characteristics of colors are not effectively utilized. Therefore, the problem cannot be solved by these methods.

EP-A-275,636 discloses full color development processes using four differently colored toners. In the toners 30% by number or less of the particles have a volume-average particle size of less than 6.35 microns and 9% by weight or less of the particles have a size above 20.2 microns.

The present invention seeks to provide a toner for full color development which has a very high light-transmitting property, and an improved light-transmitting property such that hues of respective toners overlapped at the color mingling step are sharply manifested.

The present invention also seeks to provide toners having development characteristics and transfer characteristics which are substantially conformable to one another by diminishing the differences of electric characteristics among the respective toners, in particular so that full color development having excellent image reproducibility becomes possible without reduction of the chroma or unevenness of the density in the formed image.

In accordance with one aspect of the present invention, there is provided a high transparency toner for full color development comprising a binder resin having an electroconductivity of 1.0 x 10⁻⁹ to 5.0 x 10⁻⁹ (s/cm) and magenta coloring agent particles dispersed in the binder resin, the particle size distribution of the coloring agent being such that when the toner is formed into a layer having a thickness of 0.9 »m there are fewer than 40 dispersed coloring agent particles having a size of 10 to 12.5 »m² and fewer than 20 dispersed coloring agent particles having a size of 12.5 to 15.0 »m² per 780,000 »m² of surface of the toner layer.

In accordance with another aspect of the present invention, there is provided a high transparency toner for full color development comprising a binder resin having an electroconductivity of 1·0 x 10⁻⁹ to 5·0 x 10⁻⁹ (s/cm) and cyan coloring agent particles dispersed in the binder resin, the particle size distribution of the coloring agent being such that when the toner is formed into a layer having a thickness of 0.9 »m there are fewer than 80 dispersed coloring agent particles having a size of 10 to 12.5 »m² and fewer than 50 dispersed coloring agent particles having a size of 12.5 to 15.0 »m² per 780.000 »m² of surface of the toner layer.

In accordance with still another aspect of the present invention, there is provided high transparency toner for full color development comprising a binder resin having an electroconductivity of 1·0 x 10⁻⁹ to 5·0 x 10⁻⁹ (s/cm) and yellow coloring agent particles dispersed in the binder resin, the particle size distribution of the coloring agent being such that when the toner is formed into a layer having a thickness of 0.9 »m there are fewer than 15 dispersed coloring agent particles having a size of 10 to 12.5 »m² and fewer than 10 dispersed coloring agent particles having a size of 12.5 to 15.0 »m² per 780,000 »m² of surface of the toner layer.

Fig. 1 is a characteristic curve illustrating the transmission of a conventional toner comprising a magenta coloring agent.

Fig. 2 is a characteristic curve illustrating the transmission of a toner of the present invention comprising a magenta coloring agent.

Fig. 3 is a characteristic curve illustrating the transmission of a conventional toner comprising a cyan coloring agent.

Fig. 4 is a characteristic curve illustrating the transmission of a toner of the present invention comprising a cyan coloring agent.

Fig. 5 is a characteristic curve illustrating the transmission of a conventional toner comprising a yellow coloring agent.

Fig. 6 is a characteristic curve illustrating the transmission of a toner of the present invention comprising a yellow coloring agent.

Fig. 7 is a diagram illustrating the principle of a full color development apparatus.

Factors having an influence on the transparency of the toner include the characteristics of the binder resin for example optical characteristics such as spectral reflecting and spectral transmitting properties, and the uniformity of the shape. However, it has hardly before been considered that the state of dispersion of the coloring agent in the binder resin has a significant influence on the transparency of the toner. We have now examined this dispersion and as a result have now completed the present invention.

More specifically, we have found that if the binder resin is kneaded with the coloring agent until a specific dispersion state of the coloring agent is attained and the coloring agent is uniformly dispersed in the form of predetermined fine particles, a color toner having an excellent light-transmitting property in the visible region, as not observed in conventional toners, can be obtained. The preferred dispersion state of a coloring agent and a preferred amount of the dispersed coloring agent for each of full color development toners to be overlapped, especially magenta, cyan and yellow toners, were examined. As a result, we have now completed the present invention.

A conventional organic coloring agent has a primary particle diameter of about 0.1 to 0.2 »m in the as-prepared state, but since particles are readily agglomerated in the drying step, the secondary particle size is in a broad range of from several »m to several »m. In conventional toners, a coloring agent having such a particle size is mainly dispersed in a resin.

In contrast, in the toner of the present invention, the amounts of particles having a size of 10 to 12.5 »m² and particles having a size of 12.5 to 15.0 »m are limited below certain levels. These particles, the presence of which is restricted, correspond mainly to secondary particles. The toner in which the particles are restricted has an excellent light-transmitting property in the visible region except in the wavelength absorption region of the coloring agent. We have also found that the allowable numbers of coloring agent particles having a size of 10 to 12.5 »m² and coloring agent particles having a size of 12.5 to 15.5 »m in the resin differ for magenta, cyan and yellow toners.

Fig. 1 shows the results of the examination of the transmission T (%) of a conventional toner comprising a magenta coloring agent at a wavelength in the visible region, and Fig. 2 shows the results of the examination of the transmission T (%) of a toner having a magenta coloring agent appropriately dispersed in a resin according to the present invention, at a wavelength in the visible region. As is seen from Figs. 1 and 2, these magenta toners show substantially the same absorption values at a wavelength of about 500 to 600 nm, but in other areas of the visible region (wavelengths shorter than 500 nm and longer than 600 nm), they do not absorb light but transmit it. Furthermore, in the above region the conventional toner has a poor light-transmitting property. In contrast, the magenta toner of the present invention exerts the same action as that of the conventional toner in the inherent absorption region of the coloring agent, but the toner of the present invention has an excellent light-transmitting property in other visible regions. Accordingly, the toner of the present invention is suitably used as a toner for full color development and provides an image having excellent reproducibility.

In the magenta toner of the present invention, it is important that when the toner is formed into a layer having a thickness of 0.9 »m as a measurement sample, there are fewer than 40, especially fewer than 30, dispersed coloring agent particles having a size of 10 to 12.5 »m² and fewer than 20, especially fewer than 10, dispersed coloring agent particles having a size of 12.5 to 15.0 »m² per 780,000 »m² of surface of the toner layer. If the number of coloring agent particles is within the above-mentioned range, a sufficient light-transmitting property can be obtained, but if the number of particles exceeds the above-mentioned range, the light-transmitting property is degraded. The reason why the transparency of the toner is improved by restricting the presence of coloring agent particles having such a large size has not been elucidated, but it is believed that many coloring agent particles having a primary particle size are present in the binder, they are uniformly dispersed and polymeric films of the resin wet-adhere to the entire surfaces of the coloring agent particles.

In the above-mentioned magenta toner, a quinacridone pigment is preferably used as the coloring agent. The quinacridone pigment has a good dispersibility in a resin, and the above-mentioned requirements of the numbers of particles having the above-mentioned particle sizes may be satisfied. Thus, the quinacridone pigment has a good dispersibility in a binder resin, and a toner comprising the quinacridone pigment has uniform electric characteristics and excellent light-transmitting and spectral characteristics.

Fig. 3 shows the results of the examination of the transmission T (%) of a conventional toner comprising a cyan coloring agent at a wavelength in the visible region, and Fig. 4 shows the results of the examination of the transmission T (%) of a toner having a cyan coloring agent appropriately dispersed in a resin according to the present invention, at a wavelength in the visible region. As is seen from Figs. 3 and 4, these cyan toners show substantially the same absorption values at a wavelength of about 600 to 700 nm, but in the wavelength region of about 500 nm, they do not absorb light but transmit it. Furthermore in the above region the conventional toner has a poor light-transmitting property. In contrast, the cyan toner of the present invention exerts the same action as that of the conventional toner in the inherent absorption region of the coloring agent, but the toner of the present invention has an excellent light-transmitting property in other visible regions. Accordingly, the toner of the present invention is suitably used as a toner for full color development and provides an image having excellent reproducibility.

In the cyan toner of the present invention, it is important that when the toner is formed into a layer having a thickness of 0.9 »m as a measurement sample, there are fewer than 80, especially fewer than 70, dispersed coloring agent particles having a size of 10 to 12.5 »m² and fewer than 50, especially fewer than 40, dispersed coloring agent particles having a size of 12.5 to 15.0 »m² per 780,000 »m² of surface of the toner layer. If the number of coloring agent particles is within the above-mentioned range, a sufficient light-transmitting property can be obtained, but if the number of particles exceeds the above-mentioned range, the light-transmitting property is degraded.

In the above-mentioned cyan toner, a copper phthalocyanine pigment is preferably used as the coloring agent. The copper phthalocyanine pigment has a good dispersibility in a resin, and the above-mentioned requirements of the numbers of particles having the above-mentioned particle sizes may be satisfied. Thus, the copper phthalocyanine pigment has a good dispersibility in a binder resin, and a toner comprising the copper phthalocyanine pigment has uniform electric characteristics and excellent light-transmitting characteristics.

Fig. 5 shows the results of the examination of the absorption wavelengths of a conventional toner comprising a yellow coloring agent in the visible region, and Fig. 6 shows the results of the examination of the absorption wavelengths of a toner having a yellow coloring agent appropriately dispersed in a resin according to the present invention, in the visible region. As is seen from Figs. 5 and 6, these yellow toners show substantially the same absorption values at a wavelength of about 400 nm, but in other areas of the visible region (wavelengths longer than 500 nm), they do not absorb light but transmit it. Furthermore in the above region, the conventional toner has a poor light-transmitting property. In contrast, the yellow toner of the present invention exerts the same action as that of the conventional toner in the inherent absorption region of the coloring agent, but the toner of the present invention has an excellent light-transmitting property in other visible regions. Accordingly, the toner of the present invention is suitably used as a toner for full color development and provides an image having excellent reproducibility.

In the yellow toner of the present invention, it is important that when the toner is formed into a layer having a thickness of 0.9 »m as a measurement sample, there are fewer than 15, especially fewer than 10, dispersed coloring agent particles having a size of 10 to 12.5 »m² and fever than 10, especially fever than 5, dispersed coloring agent particles having a size of 12.5 to 15.0 »m² per 780,000 »m² of surface of the toner layer. If the number of coloring agent particles is within the above-mentioned range, a sufficient light-transmitting property can be obtained, but if the number of particles exceeds the above-mentioned range, the light-transmitting property is degraded.

In the above-mentioned yellow toner, a benzidine pigment is preferably used as the coloring agent. The benzidine pigment has a good dispersibility in a resin, and the above-mentioned requirements of the numbers of particles having the above-mentioned particle sizes may be satisfied. Thus, the benzidine pigment has a good dispersibility in a binder resin, and a toner comprising the benzidine pigment has uniform electric characteristics and excellent light-transmitting characteristics.

In the present invention, it is important that the electroconductivity of the binder resin is from 1.0 x 10⁻⁹ to 5.0 x 10⁻⁹ (s/cm), and it is especially preferred that the electroconductivity is 1.0 x 10⁻⁹ to 3.0 x 10⁻⁹ (s/cm). If the electroconductivity of the binder resin is less than the above-mentioned range, a great difference of the electroconductivity is produced among toners to be overlapped, and also great differences are produced in the development and transfer characteristics. For example, as shown in Experiment 4-5 (Table 4) hereinafter, if a binder resin having a low electroconductivity of 8.9 x 10⁻¹⁰ s/cm is used, carbon black raises up the electroconductivity of the entire toner to 1.5 x 10⁻⁹ s/cm, while other toners such as cyan, magenta and yellow toners show an electroconductivity of an order of 10 x 10⁻¹⁰ s/cm, and coloring agents fail to show such a prominent increase of the electroconductivity as attained by carbon black. Therefore, differences of the electrocoductivity are produced among the overlapped toners.

In contrast, if a binder resin having an electroconductivity within the above-mentioned range is used, no difference of the electroconductivity is found among the magenta, cyan and yellow toners of the present invention, for example as shown in Experiments 4-1 and 4-2 concerning the magenta toner. If full color development is carried out using toners, among which there is no difference of electroconductivity, the development and transfer characteristics are substantially the same and excellent image reproducibility is attained. On the other hand, if the electroconductivity of the binder resin is greater than the above-mentioned range, even if charges are applied to toners, escape of the charges is delayed and the charging state becomes unstable.

If the binder resin has an electroconductivity within the above-mentioned range, the toner of the present invention has satisfactory electric characteristics, and the resin of the toner of the present invention may be the same as or different from binder resins of other toners used simultaneously with the toner of the present invention. Incidentally, it is important that each of the binder resins of other toners should satisfy the above-mentioned requirements of the electroconductivity.

In the present invention, it also is important that the melting point of the binder resin should preferably be 80 to 130°C, more preferably 90 to 110°C. If the melting point of the binder resin is within the above-mentioned range, an excellent coloring property is attained if respective toners are overlapped. If the melting point of the binder resin is above the above-mentioned range, the coloring property is degraded, and if the melting point of the binder resin is below the above-mentioned range, an offset phenomenon is sometimes caused.

The toner of the present invention will now be further described in detail.

The toner of the present invention is a toner for full color development, where the toner is overlapped on other toners differing in color on an image on a transfer sheet. The present invention is directed to a toner forming a basic color in full color development. Basic toners for full color development include four toners, that is, magenta, cyan, yellow and black toners. In full color development, these toners are developed in order in the overlapped state, and the hue and image quality of an original are reproduced. Each of these toners comprises a coloring agent and, if desired, a charge-controlling agent in a binder resin. A known toner can be further incorporated in or added to the toner.

A known resin can be used as the binder resin in the present invention, but it is important that the resin used as the binder resin should have an electroconductivity of 1.0 x 10⁻⁹ to 5.0 x 10⁻⁹ (s/cm), preferably 1.0 x 10⁻⁹ to 3.0 x 10⁻⁹ (s/cm), as pointed out hereinbefore. Moreover, a resin having an excellent light-transmitting property is preferably used. It also is important that the binder resin preferably has a melting point of 80 to 130°C, more preferably 90 to 110°C.

As the resin having such characteristics, polyester, polystyrene, polyacrylic, polyamide and polyolefin resins can be used singly or in the form of mixtures of two or more of them.

In specific examples of the polyester resin, an aromatic dicarboxylic acid or a fatty acid may be the acid component. As examples of the acid component, there can be mentioned terephthalic acid, isophthalic acid, naphthalene-dicarboxylic acid, maleic acid, fumaric acid, succinic acid, adipic acid, sebacic acid and cyclohexane-dicarboxylic acid. Terephthalic acid is mainly used. As the diol component, there can be mentioned, for example, ethylene glycol, propylene glycol, diethylene glycol, butanediol, cyclohexane dimethanol, hexylene glycol, triethylene glycol, glycerol, mannitol and pentaerythritol.

Specific examples of the styrene resin include polymers obtained by polymerizing monomers such as styrene, α-methylstyrene, vinyltoluene, α-chlorostyrene, o-chlorostyrene, m-chlorostyrene, p-chlorostyrene, ethylstyrene and divinylstyrene singly or in combination.

As the acrylic resin, there can be used, for example, polymers obtained by polymerizing monomers such as ethyl acrylate, methyl methacrylate, butyl methacrylate, 2-ethyl-hexyl methacrylate, acrylic acid and methacrylic acid singly or in combination. As the comonomer other than the above-mentioned monomers, there can be used ethylenically unsaturated acid and anhydrides thereof, such as maleic anhydride, fumaric acid, maleic acid, crotonic acid and itaconic acid.

Polymers comprising, for example, vinyl-n-butyl ether, vinylphenyl ether or vinylcyclohexanyl ether can be used a the vinyl ether resin.

Known resins derived from a diamine and a dicarboxylic acid and resins formed by polymerizing a lactam, such as nylon 6, can be used as the polyamide resin.

Polymers formed by polymerizing, for example, ethylene, propylene, butene-1, pentene-1 or methylpentene-1 can be mentioned as the olefin resin.

The foregoing resins can be used singly, or two or more can be combined so that the above-mentioned electroconductivity is attained, and the resulting mixtures can be used as the binder resin.

In the present invention , in view of the electroconductivity, light-transmitting property and melt viscosity characteristics, a polyester resin is preferably used.

The coloring agent to be contained in the coloring resin is roughly divided magenta, cyan and yellow pigments. Preferably, the coloring agent is incorporated in the binder resin in an amount of 1 to 20% by weight based on the binder resin.

As the magenta coloring agent, there can be mentioned C.I. Pigment Red 81, C.I. Pigment Red 122, C.I. Pigment Red 57, C.I. Solvent Red 49, C.I. Solvent Red 19, C.I. Solvent Red 52, C.I. Basic Red 10 and C.I. Disperse Red 15.

A quinacridone pigment is especially preferably used as the magenta coloring agent because the quinacridone pigment has good dipersibility in the binder resin. The quinacridone pigment is represented by the formula:
wherein R₁ and R₂ represent an imino group or a carbonyl group, and R₃ and R₄ represent a hydrogen atom, an alkyl group or a halogen atom.

As the cyan coloring agent, there can be mentioned C.I. Pigment Blue 15, C.I. Pigment Blue 16, C.I. Solvent Blue 25, C.I. Solvent Blue 55, C.I. Solvent Blue 70, C.I. Direct Blue 86 and C.I. direct Blue 25.

A copper phthalocyanine pigment is preferably used as the cyan coloring agent because the copper phthalocyanine pigment has good dispersibility in the binder resin. The copper phthalocyanine pigment is represented by the formula:
wherein the benzene nuclei can be substituted with an alkyl group or a halogen atom.

As the yellow coloring agent, there can be mentioned nitro pigments such as Naphthol Yellow, azo pigments such as Hansa Yellow 5G, Hansa Yellow 3G, Hansa Yellow G, Benzidine Yellow GR, Benzidine Yellow G and Vulcan Yellow 5G, inorganic pigments such as yellow iron oxide and yellow ochre, and oil-soluble dyes listed in Color Index, such as C.I. Solvent Yellow 2, C.I. Solvent Yellow 6, C.I. Solvent Yellow 14, C.I. Solvent Yellow 15, C.I. Solvent Yellow 16, C.I. Solvent Yellow 19 and C.I. Solvent Yellow 21.

Among these yellow coloring agents, an organic dye or pigment is preferably used from the viewpoint of the dispersibility in the binder resin. A benzidine pigment is especially preferably used because the dispersibility in the binder resin is very good and the pigment is dispersed in the form of very fine particles, and a yellow toner having excellent electric characteristics can be provided.

A charge-controlling agent can be incorporated into the binder resin for controlling the charging of the toner. A known charge-controlling agent can be used in the present invention. For example, there can be mentioned oil-soluble dyes such as Nigrosine Base (C.I. 50415), Oil Black (C.I. 26150) and Spiron Black, metal salts of naphthenic acid, metal soaps, metal-containing azo dyes, pyrimidine compounds and metal chelates of alkylsalicylic acids. A zinc salt or zinc complex of salicylic acid and a zinc salt or zinc complex of an alkylsalicylic acid are preferably used as the charge-controlling agent. It is preferred that the charge-controlling agent be incorporated in the binder resin in an amount of 0.5 to 5.0% by weight based on the binder resin.

The toner for full color development, prepared from the foregoing components, preferably has a particle size such that the median diameter based on the volume, measured by a Coulter Counter, is 5 to 20 »m, especially 8 to 15 »m. The flowability of the toner can be improved by sprinkling inorganic fine particles such as hydrophobic silica fine particles or organic fine particles composed of, for example, a polymer on the surface of the toner.

It is preferred that when the transmission T (%) at 550 nm of the magenta toner is lower than 2%, the transmission T (%) at 440 nm of the toner be at least 40%, especially at least 45%.

It is preferred that when the transmission T (%) at 600 nm of the cyan toner is lower than 2%, the transmission T (%) at 490 nm of the toner be at least 70%, especially at least 75%.

It is preferred that when the transmission T (%) at 400 nm of the yellow toner is lower than 2%, the transmission T (%) at 550 nm of the toner be at least 75%, especially at least 80%.

In the case where the above-mentioned toner is used as a two-component type developer by mixing it with a magnetic carrier, any known magnetic carriers used in this field can be used, but ferrite particles capable of forming a soft magnetic brush are generally preferred.

As is apparent from the foregoing description, according to the present invention, by limiting the numbers of particles having a size of 10 to 12.5 »m² and particles having a size of 12.5 to 15.0 »m² among the coloring agent particles dispersed in the binder resin to below certain values, the light-transmitting property can be improved for any of the magenta, cyan and yellow toners. Accordingly, these toners having an improved light-transmitting property are preferably used for the full color development where the toners are used in the overlapped state.

Furthermore, according to the present invention, by using a resin having an electroconductivity of 1.0 x 10⁻⁹ to 5.0 x 10⁻⁹ (s/cm) as the binder resin of the toner, the differences of electric characteristics among toners used in the overlapped state for the full color development can be diminished. If the differences of electric characteristics among the toners can be diminished, the development conditions for full color development can be made substantially the same among the toners. Therefore, the difference of the transfer quantity among the toners can be reduced and full color treatment can be performed with an excellent image reproducibility.

The present invention will now be further described in the following Examples.

### (Experiment 1)

### Experiment 1-1

### (1) Preparation of Magenta Toner

A polyester resin as the binder resin, a quinacridone pigment as the coloring agent and, optionally, a charge-controlling agent were sufficiently kneaded, pulverized and classified to obtain a toner having a particle size of 5 to 15 »m.

This kneading was conducted so that when the toner was formed into a layer having a thickness of 0.9 »m, in an area of 780,000 »m² of the formed surface of the toner, the number of coloring agent particles having a size of 10.0 to 12.5 »m² was 30 and the number of coloring agent particles having a size of 12.5 to 15.0 »m² was 10.

As shown in Table 1, the transmission T (%) of the obtained toner at 550 nm was 2% and the transmission T (%) at 440 nm was 48%. The relation between the wavelength and the transmission is shown in Fig. 2.

The above toner was mixed with a known magnetic ferrite carrier to form a two-component developer.

### (2) Preparation of Cyan Toner

The same binder resin as used for the magenta toner was used, and a copper phthalocyanine pigment was used as the coloring agent. These components were kneaded so that when the toner was formed into a layer having a thickness of 0.9 »m, in the area of 780,000 »m² of the formed surface of the toner, the number of coloring agent particles having a size of 10.00 to 12.5 »m² was 60 and the number of coloring agent particles having a size of 12.5 to 15.0 »m² was 35.

The toner was mixed with a known magnetic ferrite carrier to form a two-component developer.

### (3) Preparation of Yellow Toner

The same binder resin as used for the magenta toner was used, and a benzidine pigment was used as the coloring agent. These components were kneaded so that when the toner was formed into a layer having a thickness of 0.9 »m, in the area of 780,000 »m² of the formed surface of the toner, the number of coloring agent particles having a size of 10.00 to 12.5 »m² was 10 and the number of coloring agent particles having a size of 12.5 to 15.0 »m² was 5.

The toner was mixed with a known magnetic ferrite carrier to form a two-component developer.

Toners (1) through (3) were subjected to full color development under the same conditions shown in Table 1 and were overlapped on a transfer material. The formed image was evaluated. The results of the evaluation are shown in Table 1.

### Experiments 1-2 through 1-5

### (1) Preparation of Magenta Toner

In the same manner as described in Experiment 1-1, a toner having a particle size of 5 to 15 »m was prepared, and the number of coloring agent particles and the transmission of the toner were as shown in Table 1.

The obtained toner was formed in a two-component developer in the same manner as described in Experiment 1-1.

The same cyan and yellow toners as used in Experiment 1-1 were used.

The image formed by using these toners was evaluated in the same manner as described in Experiment 1-1. The results of the evaluation are shown in Table 1.

### Experiment 1-6

### (1) Preparation of Magenta Toner

A polyester resin as the binder resin, a quinacridone pigment as the coloring agent and, optionally, a charge-controlling agent were sufficiently kneaded, pulverized and classified to obtain a toner having a particle size of 5 to 15 »m.

This kneading was conducted so that when the toner was formed into a layer having a thickness of 0.9 »m, in the area of 780,000 »m² of the formed surface of the toner, the number of coloring agent particles having a size of 10.0 to 12.5 »m² was 120 and the number of coloring agent particles having a size of 12.5 to 15.0 »m² was 80.

The transmission T (%) of the obtained toner at 550 nm was 1.5% and the transmission T (%) at 440 nm was 20%. The relation between the wavelength and the transmission is shown in Fig. 1.

The image formed by using this magenta toner and the same cyan and yellow toners as used in Experiment 1-1 was evaluated in the same manner as described in Experiment 1-1. The obtained image was dark and had extremely poor transparency and sharpness.

### (Experiment 2)

### Experiment 2-1

### (1) Preparation of Cyan Toner

A polyester resin as the binder resin, a copper phthalocyanine pigment as the coloring agent and, optionally, a charge-controlling agent were sufficiently kneaded, pulverized and classified to obtain a toner having a particle size of 8 to 15 »m.

This kneading was conducted so that when the toner was formed into a layer having a thickness of 0.9 »m, in the area of 780,000 »m² of the formed surface of the toner, the number of coloring agent particles having a size of 10.0 to 12.5 »m² was 60 and the number of coloring agent particles having a size of 12.5 to 15.0 »m² was 35.

As shown in Table 2, the transmission T (%) of the obtained toner at 600 nm was 1.0% and the transmission T (%) at 490 nm was 76%. The relation between the wavelength and the transmission is shown in Fig. 4.

The above toner was mixed with a known magnetic ferrite carrier to form a two-component developer.

### (2) Preparation of Yellow Toner

The same binder resin as used for the cyan toner was used, and a benzidine pigment was used as the coloring agent. These components were kneaded so that when the toner was formed into a layer having a thickness of 0.9 »m, in the area of 780,000 »m² of the formed surface of the toner, the number of coloring agent particles having a size of 10.00 to 12.5 »m² was 10 and the number of coloring agent particles having a size of 12.5 to 15.0 »m² was 5.

The toner was mixed with a known magnetic ferrite carrier to form a two-component developer.

### (3) Preparation of Magenta Toner

The same binder resin as used for the cyan toner was used, and a quinacridone pigment was used as the coloring agent. These components were kneaded so that when the toner was formed into a layer having a thickness of 0.9 »m, in the area of 780,000 »m² of the formed surface of the toner, the number of coloring agent particles having a size of 10.00 to 12.5 »m² was 30 and the number of coloring agent particles having a size of 12.5 to 15.0 »m² was 10.

The toner was mixed with a known magnetic ferrite carrier to form a two-component developer.

Toners (1) through (3) were subjected to full color development under same conditions shown in Table 2 and were overlapped on a transfer material. The formed image was evaluated. The results of the evaluation are shown in Table 2.

### Experiments 2-2 through 2-3

### (1) Preparation of Cyan Toner

In the same manner as described in Experiment 2-1, a toner having a particle size of 8 to 15 »m was prepared, and the number of coloring agent particles and the transmission of the toner were as shown in Table 2.

The obtained toner was formed in a two-component developer in the same manner as described in Experiment 2-1.

The same magenta and yellow toners as used in Experiment 2-1 were used.

The image formed by full color development using these toners was evaluated in the same manner as described in Experiment 2-1. The results of the evaluation are shown in Table 2.

### Experiment 2-4

### (1) Preparation of Cyan Toner

A polyester resin as the binder resin, a copper phthalocyanine pigment as the coloring agent and, optionally, a charge-controlling agent were sufficiently kneaded, pulverized and classified to obtain a toner having a particle size of 8 to 15 »m.

This kneading was conducted so that when the toner was formed into a layer having a thickness of 0.9 »m, in the area of 780,000 »m² of the formed surface of the toner, the number of coloring agent particles having a size of 10.0 to 12.5 »m² was 110 and the number of coloring agent particles having a size of 12.5 to 15.0 »m² was 80.

The transmission T (%) of the obtained toner at 600 nm was 0.5% and the transmission T (%) at 490 nm was 64%. The relation between the wavelength and the transmission is shown in Fig. 3.

The image formed by using this cyan toner and the same magenta and yellow toners as used in Experiment 2-1 was evaluated in the same manner as described in Experiment 2-1. The obtained image was dark and had extremely poor transparency and sharpness.

### Experiment 2-5

### (1) Preparation of Cyan Toner

A cyan toner was prepared in the same manner as described in Experiment 2-4 except that kneading was carried out so that when the toner was formed into a layer having a thickness of 0.9 »m, in the area of 780,000 »m² of the formed surface of the toner, the number of coloring agent particles having a size of 10.0 to 12.5 »m² was 78 and the number of coloring agent particles having a size of 12.5 to 15.0 »m² was 53.

This cyan toner and the same magenta and yellow toners as used in Experiment 2-1 were subjected to full color development and were overlapped on a transfer material to form an image. The formed image was evaluated. The image had poor sharpness.

### (Experiment 3)

### Experiment 3-1

### (1) Preparation of Yellow Toner

A polyester resin as the binder resin, a benzidine pigment as the coloring agent and, optionally, a charge-controlling agent were sufficiently kneaded, pulverized and classified to obtain a toner having a particle size of 5 to 15 »m.

This kneading was conducted so that when the toner was formed into a layer having a thickness of 0.9 »m, in the area of 780,000 »m² of the formed surface of the toner, the number of coloring agent particles having a size of 10.0 to 12.5 »m² was 10 and the number of coloring agent particles having a size of 12.5 to 15.0 »m² was 6.

As shown in Table 3, the transmission T (%) of the obtained toner at 400 nm was 2% and the transmission T (%) at 550 nm was 80%. The relation between the wavelength and the transmission is shown in Fig. 6.

The above toner was mixed with a known magnetic ferrite carrier to form a two-component developer.

### (2) Preparation of Magenta Toner

The same binder resin as used for the yellow toner was used, and a quinacridone pigment was used as the coloring agent. These components were kneaded so that when the toner was formed into a layer having a thickness of 0.9 »m, in the area of 780,000 »m² of the formed surface of the toner, the number of coloring agent particles having a size of 10.00 to 12.5 »m² was 30 and the number of coloring agent particles having a size of 12.5 to 15.0 »m² was 10.

The toner was mixed with a known magnetic ferrite carrier to form a two-component developer.

### (3) Preparation of Cyan Toner

The same binder resin as used for the yellow toner was used, and a copper phthalocyanine pigment was used as the coloring agent. These components were kneaded so that when the toner was formed into a layer having a thickness of 0.9 »m, in the area of 780,000 »m² of the formed surface of the toner, the number of coloring agent particles having a size of 10.00 to 12.5 »m² was 60 and the number of coloring agent particles having a size of 12.5 to 15.0 »m² was 35.

The toner was mixed with a known magnetic ferrite carrier to form a two-component developer.

Toners (1) through (3) were subjected to full color development under same conditions shown in Table 3 and were overlapped on a transfer material. The formed image was evaluated. The results of the evaluation are shown in Table 3.

### Experiments 3-2 through 3-4

### (1) Preparation of Yellow Toner

In the same manner as described in Experiment 3-1, a toner having a particle size of 5 to 15 »m was prepared, and the number of coloring agent particles and the transmission of the toner were as shown in Table 3.

The obtained toner was formed in a two-component developer in the same manner as described in Experiment 3-1.

The same magenta and cyan toners as used in Experiment 3-1 were used.

The image formed by full color development using these toners was evaluated in the same manner as described in Experiment 3-1. The results of the evaluation of the image of the toners overlapped on a transfer material are shown in Table 3.

### Experiment 3-5

### (1) Preparation of Yellow Toner

A polyester resin as the binder resin, a benzidine pigment as the coloring agent and, optionally, a charge-controlling agent were sufficiently kneaded, pulverized and classified to obtain a toner having a particle size of 5 to 15 »m.

This kneading was conducted so that when the toner was formed into a layer having a thickness of 0.9 »m, in the area of 780,000 »m² of the formed surface of the toner, the number of coloring agent particles having a size of 10.0 to 12.5 »m² was 30 and the number of coloring agent particles having a size of 12.5 to 15.0 »m² was 25.

The transmission T (%) of the obtained toner at 400 nm was 2.0% and the transmission T (%) at 550 nm was 62%. The relation between the wavelength and the transmission is shown in Fig. 5.

The image formed by full color development using this yellow toner and the same magenta and cyan toners as used in Experiment 3-1 was evaluated in the same manner as described in Experiment 3-1. The obtained image had an unevendensity and poor the sharpness.

### (Experiment 4)

### Experiment 4-1

A toner having an average particle size of 10 »m and an electroconductivity of 2.5 x 10⁻⁹ (s/cm) was prepared by kneading 100 parts by weight of a polyester resin having an electroconductivity of 2.5 x 10⁻⁹ (s/cm) and a melting point of 90° as the binder resin and 4.0 parts by weight of a quinacridone pigment as the coloring agent so that when the obtained toner was formed in a layer having a thickness of 0.9 »m, in the area of 780,000 »m² of the formed surface of the toner, the number of dipsersed particles having a size of 10 to 12.5 »m² was 29 and the number of dispersed particles having a size of 12.5 to 15.0 »m² was 8.

A toner having an average particle size of 10 um and an electroconductivity of 2.6 x 10⁻⁹ (s/cm) was prepared by kneading 100 parts by weight of the same binder resin as used above and 3.0 parts by weight of a benzidine pigment as a yellow coloring agent so that when the obtained toner was formed into a layer having a thickness of 0.9 »m, in the area of 780,000 »m² of the formed surface of the toner, the number of pigment particles having a size of 10.0 to 12.5 »m² was 10 and the number of particles having a size of 12.5 to 15.0 »m² was 5.

A toner having an average particle size of 10 »m and an electroconductivity of 2.5 x 10⁻⁹ (s/cm) was prepared by kneading 100 parts by weight of the same binder resin as described above and 4.0 parts by weight of a copper phthalocyanine as a cyan coloring pigment so that when the obtained toner was formed in a layer having a thickness of 9 »m, in the area of 780,000 »m² of the formed surface of the toner, the number of dispersed pigment particles having a size of 10.0 to 12.5 »m² was 58 and the number of dispersed pigment particles was 36.

A black toner having an electroconductivity of 2.7 x 10⁻⁹ (s/cm) was prepared by using 100 parts by weight of the binder resin and 4 parts by weight of carbon black according to customary procedures.

The foregoing toners were independently mixed with a known ferrite carrier to prepare respective color developers. These developers were subjected to full color development under same developing conditions and were overlapped on a transfer material to obtain a full color image. With respect to each developed toner, the toner transfer efficiency was determined by using an A-4 original having an image area ratio of 20%. The obtained results are shown in Table 4.

### Experiments 4-2 through 4-5

The experiments were carried out in the same manner as described in Experiment 4-1 except that the electroconductivity and melting temperature of the binder resin, the magenta coloring agent and the dispersion states of the coloring agents in the toners were changed as shown in Table 4. The obtained results are shown in Table 4.

From the results obtained in Experiments 4-1 and 4-2, it is seen that in the magenta toner of the present invention, the developing and transfer characteristics can be made almost equal to those of other color toners and that this magenta toner has excellent transparency and coloring properties. Therefore a sharp full color image can be provided without any density unevenness.

### (Experiment 5)

### Experiments 5-1 through 5-5

Experiments were carried out in the same manner as described in Experiment 4-1 except that the electroconductivity and melting point of the binder resin, the cyan coloring agent and the dispersion states of the coloring agents in the toners were changed as shown in Table 5. The obtained full color images were evaluated. The obtained results are shown in Table 5.

### (Experiment 6)

### Experiments 6-1 through 6-5

Various toners were prepared in the same manner as described in Experiment 5-1 except that the electrocoductivity and melting point of the binder resin, the cyan coloring agent and the dispersion states of the coloring agents in the toners were changed as shown in Table 6, and images formed by full color development using these toners were evaluated. The obtained results are shown in Table 6.

From the results obtained in Experiments 5-1 and 5-2, it is seen that in the cyan toner of the present invention, the developing and transfer characteristics can be made substantially equal to those of other color toners and that this cyan toner has excellent transparency and coloring properties. Therefore, a sharp full color image can be provided without any density unevenness.

From the results obtained in Experiments 6-1 and 6-2, it is seen that in the yellow toner of the present invention, the developing and transfer characteristics can be made substantially equal to those of other color toners and that this cyan toner has excellent transparency and coloring properties. Therefore, a sharp full color image can be provided without any density unevenness.

## Claims

1. A high transparency toner for full colour development comprising a binder resin having an electroconductivity of 1.0 x 10⁻⁹ to 5.0 x 10⁻⁹ (s/cm) and magenta colouring agent particles dispersed in the binder resin, the particle size distribution of the colouring agent being such that when the toner is formed into a layer having a thickness of 0.9 »m there are fewer than 40 dispersed colouring agent particles having a size of 10 to 12.5 »m² and fewer than 20 dispersed colouring agent particles having a size of 12.5 to 15.0 »m² per 780,000 »m² of surface of the toner layer.

2. A toner according to claim 1 wherein the colouring agent is a quinacridone pigment.

3. A high transparency toner for full colour development comprising a binder resin having an electroconductivity of 1.0 x 10⁻⁹ to 5.0 x 10⁻⁹ (s/cm) and cyan colouring agent particles dispersed in the binder resin, the particle size distribution of the colouring agent being such that when the toner is formed into a layer having a thickness of 0.9 »m there are fewer than 80 dispersed colouring agent particles having a size of 10 to 12.5 »m² and fewer than 50 dispersed colouring agent particles having a size of 12.5 to 15.0 »m² per 780,000 »m² of surface of the toner layer.

4. A toner according to claim 3 wherein the colouring agent is a copper phthalocyanine pigment.

5. A high transparency toner for full colour development comprising a binder resin having an electroconductivity of 1.0 x 10⁻⁹ to 5.0 x 10⁻⁹ (s/cm) and yellow colouring agent particles dispersed in the binder resin, the particle size distribution of the colouring agent being such that when the toner is formed into a layer having a thickness of 0.9 »m there are fewer than 15 dispersed colouring agent particles having a size of 10 to 12.5 »m² and fewer than 10 dispersed colouring agent particles having a size of 12.5 to 15.0 »m² per 780,000 »m² of surface of the toner layer.

6. A toner according to claim 5 wherein the colouring agent is a benzidine pigment.

7. A toner according to any one of claims 1 to 6 wherein the melting point of the binder resin is 80 to 130°C.

8. Use of a toner according to any one of claims 1 to 7 for full colour development.

9. Use of a magenta toner according to claim 1 or claim 2 and a cyan toner according to claim 3 or claim 4 and a yellow toner according to claim 5 or claim 6 for full colour development.

## Patentansprüche

1. Ein Toner mit hoher Transparenz zur Entwicklung der vollen Farbe bestehend aus einem Bindeharz mit einer elektrischen Leitfähigkeit von 1,0 x 10⁻⁹ bis 5,0 x 10⁻⁹ (s/cm) und Partikeln eines Magentafarbstoffs, die in dem Bindeharz dispergiert sind, die Partikelgrößenverteilung des Farbstoffs ist so, daß, wenn der Toner zu einer Schicht mit einer Dicke von 0,9 »m geformt wird, dann weniger als 40 dispergierte Farbstoffpartikel mit einer Größe von 10 bis 12,5 »m² und weniger als 20 dispergierte Farbstoffpartikel mit einer Größe von 12,5 bis 15,0 »m² pro 780000 »m² der Oberfläche der Tonerschicht vorhanden sind.

2. Toner nach Anspruch 1, bei dem der Farbstoff ein Chinacridinpigment ist.

3. Ein Toner mit hoher Transparenz zur Entwicklung der vollen Farbe bestehend aus einem Bindeharz mit einer elektrischen Leitfähigkeit von 1,0 x 10⁻⁹ bis 5,0 x 10⁻⁹ (s/cm) und Partikeln eines Cyanfarbstoffs, die in dem Bindeharz dispergiert sind, die Partikelgrößenverteilung des Farbstoffs ist so, daß, wenn der Toner zu einer Schicht mit einer Dicke von 0,9 »m geformt wird, dann weniger als 80 dispergierte Farbstoffpartikel mit einer Größe von 10 bis 12,5 »m² und weniger als 50 dispergierte Farbstoffpartikel mit einer Größe von 12,5 bis 15,0 »m² pro 780000 »m² der Oberfläche der Tonerschicht vorhanden sind.

4. Toner nach Anspruch 3, bei dem der Farbstoff ein Kupferphthalocyaninpigment ist.

5. Ein Toner mit hoher Transparenz zur Entwicklung der vollen Farbe bestehend aus einem Bindeharz mit einer elektrischen Leitfähigkeit von 1,0 x 10⁻⁹ bis 5,0 x 10⁻⁹ (s/cm) und Partikeln eines gelben Farbstoffs, die in dem Bindeharz dispergiert sind, die Partikelgrößenverteilung des Farbstoffs ist so, daß, wenn der Toner zu einer Schicht mit einer Dicke von 0,9 »m geformt wird, dann weniger als 15 dispergierte Farbstoffpartikel mit einer Größe von 10 bis 12,5 »m² und weniger als 10 dispergierte Farbstoffpartikel mit einer Größe von 12,5 bis 15,0 »m² pro 780000 »m² der Oberfläche der Tonerschicht vorhanden sind.

6. Toner nach Anspruch 5, bei dem der Farbstoff ein Benzidinpigment ist.

7. Toner nach irgendeinem der vorherigen Ansprüche 1 bis 6, bis dem der Schmelzpunkt des Bindeharzes 80 bis 130 °C beträgt.

8. Verwendung eines Toners nach irgendeinem der vorherigen Ansprüche 1 bis 7 zur Entwicklung der vollen Farbe.

9. Verwendung eines Magentatoners nach Anspruch 1 oder Anspruch 2 und eines Cyantoners nach Anspruch 3 oder Anspruch 4 und eines Gelbtoners nach Anspruch 5 oder Anspruch 6 zur Entwicklung der vollen Farbe.

## Revendications

1. Un toneur à haute transparence pour le développement à pleine couleur comprenant une résine de liaison ayant une conductibilité électrique de 1,0 x 10⁻⁹ à 5,0 x 10⁻⁹ (s/cm) et des particules d'agent colorant magenta dispersées dans la résine de liaison, la distribution des dimensions particulaires de l'agent colorant étant telle que, lorsque le toneur est formé en une couche ayant une épaisseur de 0,9 », il y ait moins de 40 particules d'agent colorant dispersées ayant une dimension de 10 à 12,5 »² et moins de 20 particules d'agent colorant dispersées ayant une dimension de 12,5 à 15,0 »² par 780 000 »² de surface de la couche de toneur.

2. Un toneur selon la revendication 1 dans lequel l'agent colorant est un pigment de quinacridone.

3. Un toneur à haute transparence pour le développement à haute couleur comprenant une résine de liaison ayant une conductibilité électrique de 1,0 x 10⁻⁹ à 5,0 x 10⁻⁹ (s/cm) et des particules d'agent colorant cyan dispersées dans la résine de liaison, la distribution des dimensions particulaires de l'agent colorant étant telle que, lorsque le toneur est formé en une couche ayant une épaisseur de 0,9 », il y ait moins de 80 par ticules d'agent colorant dispersées ayant une dimension de 10 à 12,5 »² et moins de 50 particules d'agent colorant dispersées ayant une dimension de 12,5 à 15,0 »² par 780 000 »² de surface de la couche de toneur.

4. Un toneur selon la revendication 3 dans lequel l'agent colorant est un pigment de phtalocyanine de cuivre.

5. Un toneur à haute transparence pour le développement à pleine couleur comprenant une résine de liaison ayant une conductibilité électrique de 1,0 x 10⁻⁹ à 5,0 x 10⁻⁹ (s/cm) et des particules d'agent colorant jaune dispersées dans la résine de liaison, la distribution des dimensions particulaires de l'agent colorant étant telle que, lorsque le toneur est formé en une couche ayant une épaisseur de 0,9 », il y ait moins de 15 particules d'agent colorant dispersées ayant une dimension de 10 à 12,5 »² et moins de 10 particules d'agent colorant dispersées ayant une dimension de 12,5 à 15,0 »² par 780 000 »² de surface de la couche de toneur.

6. Un toneur selon la revendication 5 dans lequel l'agent colorant est un pigment de benzidine.

7. Un toneur selon l'une ou l'autre des revendications 1 à 6 dans lequel le point de fusion de la résine de liaison est de 80 à 130°C.

8. L'utilisation d'un toneur selon l'une ou l'autre des revendications 1 à 7 pour le développement à pleine couleur.

9. L'utilisation d'un toneur magenta selon la revendication 1 ou la revendication 2 et d'un toneur cyan selon la revendication 3 ou la revendication 4 et d'un toneur jaune selon la revendication 5 ou la revendication 6 pour le développement à pleine couleur.
